

A. E. GREENE.

METHOD OF PRODUCING REFINED METALS AND ALLOYS.

APPLICATION FILED JULY 22, 1908.

1,034,785.

Patented Aug. 6, 1912



Witnesses:

Irving MacDonald  
McGilland Young.

Inventor:

Albert E. Greene,  
By Barton, Tanner & Folk,  
Atty's.

# UNITED STATES PATENT OFFICE.

ALBERT E. GREENE, OF CHICAGO, ILLINOIS, ASSIGNOR TO AMERICAN ELECTRIC SMELTING AND ENGINEERING COMPANY, OF ST. LOUIS, MISSOURI, A CORPORATION OF MISSOURI.

## METHOD OF PRODUCING REFINED METALS AND ALLOYS.

1,034,785.

Specification of Letters Patent.

Patented Aug. 6, 1912.

Application filed July 22, 1908. Serial No. 444,740.

To all whom it may concern:

Be it known that I, ALBERT E. GREENE, a citizen of the United States, residing at Chicago, in the county of Cook and State of Illinois, have invented certain new and useful Improvements in Methods of Producing Refined Metals and Alloys, of which the following is a full, clear, concise, and exact description.

10 My invention relates to a process of refining or otherwise treating metals or alloys of metals.

More specifically it relates to a process by which sulfur and phosphorus, or either of 15 said elements may be eliminated or separated from the mixture of elements, thereby leaving the remaining constituent or constituents of the mixture in a refined condition.

20 In metal refining processes based upon the oxidation of the impurity to be eliminated, the refining of the metal is usually accompanied by a greater or less oxidation of the metal itself. Such undesired oxidation of the metal results in a partial loss of 25 the metal and is also an actual hindrance to the practice of the process, since the presence of the metallic oxid in the slag interferes with the removal of certain impurities, such 30 as sulfur, which would otherwise be taken up by the slag. In the Heroult steel process designed to overcome these objections the removal of phosphorus from the bath is likewise accompanied by the presence of iron 35 oxid in the slag, but such iron oxid may be deoxidized by means of calcium carbide formed from the lime slag employed. After the elimination of phosphorus and the deoxidation of the iron oxid the sulfur in the 40 bath may be removed by a separate washing process with a lime slag.

45 My invention contemplates the formation of a compound of the elements to be eliminated from the material under treatment, without any attendant formation of undesired compounds of the elements to be retained.

50 My invention contemplates, in the more specific application of the process, the oxidation and the resultant removal of phosphorus from a metallic mixture without the

usual detrimental oxidation of the metal itself or other elements which it is desired to retain.

In certain cases my invention contemplates dispensing with the usual slag-forming flux, as, for example, where the oxidized impurity passes off in the form of gas, or where the temperature of the bath is such that the oxidized impurity is not susceptible to subsequent reduction by the metal of the bath.

In certain other cases my invention contemplates the use of a slag-forming flux for removing the oxidized phosphorus and 65 also for simultaneously removing sulfur from the bath.

One feature of my invention consists in a combined regulation of the temperature of the material which is under treatment 70 and of the pressure of dissociation of the treating agent employed. In case the treating agent is oxygen or an oxygen compound, this feature of the invention consists in the combined regulation of the temperature 75 of the material under treatment and of the oxygen pressure of the oxidizing agent which is added to or, where a gaseous agent is employed, which is forced into contact with the treated material. More specifically, this latter feature of my invention consists in maintaining the temperature of a metallic bath at a point where the oxygen pressure of the oxid of phosphorus is below 80 the oxygen pressure of any oxid which is capable of being formed from the metal or metals to be retained in the bath, and, under such temperature conditions, introducing into the bath an oxidizing agent whose oxygen pressure is above that of the oxid 85 of the substance to be eliminated but below that of the oxid which would result from the combination of oxygen with the metal or metals to be retained in the bath. In other words, the treating agent has an 90 oxygen pressure which causes it to act as an oxidizing agent for the element or elements which it is desired to eliminate from the bath but which causes it to act as a reducing agent for the oxides of such element or elements as it is desired to retain in the bath.

Another feature of my invention appli-

2  
cable to particular conditions consists in a combined regulation of the temperature of the materials under treatment and of the pressure, within the furnace chamber, of the gases resulting from the reaction, thus so controlling the pressure of dissociation of the materials under treatment and of the products resulting from the treatment as to produce conditions favorable to the elimination of an undesired element from the material under treatment.

These and other features of my invention may be more readily understood by reference to the accompanying drawings, in which—

Figure 1 is a plan view of an electric refining furnace which represents one type of furnace in connection with which the process of my invention may be practised; Fig. 2 is a sectional view on the line 2—2 of Fig. 1; Fig. 3 is a sectional view on the line 3—3 of Fig. 1; and Fig. 4 is a diagram showing the characteristic curves of oxygen pressure for the oxids of two elements, for example, iron and phosphorus, as they lie relatively to each other at different temperatures.

I have discovered that in the case of certain elements, each susceptible to oxidation, either of them may serve as a reducing agent for the oxid of the other, according to the temperatures maintained. This is due to the fact that the relative, as well as the actual affinities of two substances for oxygen may vary for different temperatures.

The pressure of dissociation of a compound, which pressure in the case of an oxygen-bearing compound is designated the oxygen pressure, normally increases with the temperature. Since the rate of increase varies with different compounds, it happens that of two compounds their relative oxygen pressures may be changed or even reversed by variation in temperature, such variation, of course, affecting the relative affinities of the elements of the compounds for oxygen. For example, at a given temperature silicon may have such a relatively high affinity for oxygen as to serve as a reducing agent for iron oxid, whereas at a different temperature the reverse may be true, the metallic iron then serving as a reducing agent for the oxid of silicon.

I have discovered that by suitably regulating the temperature of a mixture or compound containing two elements having the above-described characteristics, and by subjecting the mixture or compound to the action of an oxidizing agent whose oxygen pressure is between the two oxygen pressures corresponding to the oxygen pressure of the oxids of the elements of the mixture or compound, I can thereby oxidize that element having the lower oxygen pressure without oxidizing the element having the higher oxygen pressure. This method of

oxidizing one element of a mixture without the oxidation of any other element or elements thereof is based upon the above-mentioned facts relative to the pressure of dissociation of oxids or, in other words, to the oxygen pressure of oxids.

From the foregoing it appears that for every temperature there is a definite oxygen pressure for any given oxid below which pressure the oxid cannot form from its elements. It further follows that the series of points representing the oxygen pressures of a given oxid for different temperatures form a curve, which curve is different for different elements. Within the working range of furnace temperatures, these curves for certain pairs of elements may even cross each other. At the point of intersection of the two curves the relative affinities of the two elements for oxygen are reversed. The temperature at which two curves, each representing the pressure of dissociation of a given element with respect to a third element, intersect I designate as the critical temperature of one element with respect to the other. At said point each of said elements has an equal affinity for the third element. For example, Fig. 4 shows diagrammatically the characteristic curves of oxygen pressure for oxid of iron ( $FeO$ ) and phosphoric oxid ( $P_2O_5$ ). At the temperature corresponding to the point of intersection  $a$  of the two curves, that is, at the critical temperature of iron and phosphorus with respect to each other, which critical temperature is above  $1700^{\circ} C.$ , the oxygen pressures  $FeO$  and  $P_2O_5$  are equal, and the two elements, iron and phosphorus, have an equal affinity for oxygen. At any temperature lower than the critical temperature, the oxygen pressure of  $FeO$  is greater than the oxygen pressure of  $P_2O_5$ . Hence if an oxidizing agent having itself an oxygen pressure intermediate to those of  $FeO$  and  $P_2O_5$  be introduced into a mixture of iron and phosphorus, such oxidizing agent will act as a carrier of oxygen to the element having the lower oxygen pressure, but not for the element having the higher oxygen pressure.

The oxygen pressure at any given temperature of any given oxidizing agent, may readily be ascertained. In the case of a gaseous agent, or an agent which may assume a gaseous state, the pressure of dissociation thereof is dependent on both the temperature and the pressure or degree of compression of the gas. The effect of pressure on a gas giving oxygen by dissociation, as, for example,



is the opposite to that due to temperature; the former lowering and the latter raising the oxygen pressure of the gas. The pres-

sure of oxygen in a gas may be further regulated by mixing with the gas another gas, as for instance a gas having a different oxygen pressure. The amount of the different constituents of the mixed gas and the degree of pressure of the gaseous mixture may be regulated to obtain the best results at the temperature at which it is desirable to practice the process.

10 The oxygen pressure of air is the actual pressure due to the oxygen constituent thereof and is approximately one-fifth of an atmosphere. The oxygen pressure of carbon dioxid ( $\text{CO}_2$ ) is the actual partial pressure of the available oxygen at the working temperature, and is much lower than that of air. The oxygen pressure of carbon monoxid ( $\text{CO}$ ) under atmospheric pressure is exceedingly low. In case a gaseous oxidizing agent is desired having an oxygen pressure greater than that of carbon dioxid, such agent may be obtained by mixing air and carbon dioxid and properly regulating the relative amounts of each, and a gaseous mixture may thus be obtained having any desired oxygen pressure between that of air as a maximum and that of carbon dioxid as a minimum. Other gases, one at least of which contains oxygen, may be mixed so

30 as to give the desired result.

The oxygen pressure of a gaseous compound, it will be understood, is the actual pressure of the uncombined oxygen and of the oxygen made available by the disassociation of oxygen compounds. The total oxygen thus available for forming new combinations is a definite proportion of the entire volume of the gas, and hence the oxygen pressure is a definite percentage of the entire working pressure of the gas. The method of calculating oxygen pressure is well known and forms no part of my present invention. In a general way, to ascertain the percentage of this available oxygen, I employ tables similar to those disclosed in Nernst's *Theoretical Chemistry*, 4th edition, (1904) pages 444-445.

50 The method which I preferably employ for obtaining a gaseous agent having the desired oxygen pressure consists as above set forth in properly mixing two or more gases one at least of which contains oxygen. The mixing is preferably done by blowing each gas from a separate engine or compressor into a common receiver or pipe and regulating the speed of each unit to furnish the desired amount of each gaseous constituent of the mixture. Such apparatus is shown in the drawings, in which the blowers 1, 2

55 60 communicate with a common receiver or pipe 3.

The process of my invention may be practised with the usual well-known types of furnaces, heated in any desired manner, as

65 70 75 80 85 90 which the heat produced by the oxidation of the element eliminated serves, with or without external heat, to maintain the required temperature of the mixture under treatment. I prefer, however, to use an electric furnace in general similar to the well-known Heroult tilting furnace. Such furnace is shown in the drawings, and consists of a crucible 4 closed by a cover 5 provided with a chimney 6. The electrodes 7, 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390

The furnace is provided with a spout 8 for running off the metal on tilting the furnace. The furnace may be provided with a charging opening closed by a door 9. The electrodes may consist of the usual carbon electrodes. The furnace is provided above the base of the crucible with openings for receiving twyers 10, which communicate in the usual way with the pipe 3. The twyers preferably dip down into the molten bath 11.

Any suitable source of electric current may be employed, the connections of the electrodes in the circuit being made in a manner well understood by those skilled in the art.

In order to more clearly set forth my invention, I will describe in detail one of the applications of my process, and for that purpose will describe the operation for the removal of phosphorus and sulfur from steel.

Molten metal containing phosphorus and sulfur which might come, for example, from an acid converter is charged into the furnace through the charging opening. The temperature of the bath is regulated by regulating the flow of the electric current to the proper point for the most efficient elimination of phosphorus without appreciable oxidation of the iron of the bath. In general, it is desirable that this temperature be as far from the critical temperature of phosphorus and iron as is practicable in order to obviate the possibility of detrimental oxidation of the iron.

A basic lime flux 12 is preferably melted on top of the bath 11. This slag is preferably basic enough to take up the phosphorus and sulfur, but not more so than is necessary, in order that the electric energy required to melt it may be as small as possible. Gas of proper oxygen pressure for selectively oxidizing the phosphorus without oxidizing the iron is supplied from the pipe 3, 120 and is blown through the twyers 10 into contact with the bath 11. This causes an oxidation of the phosphorus into phosphoric oxid,  $\text{P}_2\text{O}_5$ , which is taken up by the basic slag. Since the oxidizing gas causes no oxidation of the iron, the absence of iron oxid in the slag permits of the slag also serving to eliminate the sulfur.

By practising the process as thus described, the metal cannot be "overblown"

if the proper conditions are maintained. In some cases, however, it may be desirable from a commercial standpoint to lessen the time required for practising the process at the expense of a slight loss of iron. Hence 5 I do not wish to be understood as limiting my process to conditions under which the oxidation of the iron is entirely prevented. It suffices if the conditions are such that no 10 detrimental oxidation of the iron takes place.

If the oxidation of the iron is so small as not to seriously interfere with the removal of other impurities, such practice of the process is within the scope of this invention. 15 The oxidizing action is continued until a test sample of the material under treatment shows that the metal has been sufficiently refined. The slag and metal may then be separated in the usual manner.

In practice I may employ as the oxidizing 20 agent carbon dioxid mixed with air, the oxygen pressure of such mixture being regulated with respect to the oxygen pressure of FeO and  $P_2O_5$  in the manner hereinbefore described, that is by adding to the mixture of carbon dioxid and air a gas, such as carbon monoxid, that will render the mixture an oxidizing agent for phosphorus and at the same time a reducing agent for the oxids 25 of iron at the temperature at which the material under treatment is maintained. The CO<sub>2</sub> gas may be obtained from any desired source. In practice I have found that satisfactory results may be attained by employing the stack gases from blast furnaces 30 and modifying such gases, as may be necessary, to provide the required oxygen pressure of the gaseous treating agent.

By properly regulating the oxygen pressure of the gaseous mixture employed, the oxygen available for oxidizing purposes is used up in oxidizing the element eliminated from the bath. Hence, the resultant gas coming from the reaction constitutes a non- 40 oxidizing or even a reducing atmosphere in the refining chamber, the CO<sub>2</sub> gas being reduced by the reaction to CO gas. This non-oxidizing or reducing atmosphere in the chamber containing the carbon electrodes is 45 effective in protecting them from otherwise rapid oxidation and also in protecting the molten metal.

The use of a lime flux as above set forth is preferable, for the reason that with a flux to 50 take up the oxidized phosphorus it is possible to work nearer to the critical temperature of phosphorus and iron and also for the reason that the lime flux will at the same time eliminate sulfur from the bath.

In the above-described application of my 60 process to the production of steel, I can eliminate the possibility of "overblowing" or oxidizing the iron. I thereby largely eliminate the necessity of a deoxidizing 65 process like that of the Heroult process in

which the deoxidizing agent calcium carbid is expensive in time, material and electric energy.

The effect of the pressure in the furnace chamber of the gaseous body liberated there-in tends to retard the action taking place in the body of the material. As a rule, owing to the free escape of the gases through the chimney of the furnace, such pressure of the gases resulting from the reaction, is negligible. However, in certain cases the process may be advantageously expedited by reducing the pressure in the furnace chamber. I may, therefore, employ a suction fan 12, as shown in Fig. 3, for removing through the 70 chimney or escape vent 6 of the furnace the gases as they are formed, thus maintaining the atmosphere within the chamber under a reduced pressure more favorable to the practice of the process. 75

With reference to the practice of my process in general, it is to be understood that it is not limited to any particular method of regulating the temperature of the substance under treatment, or of subjecting the same 80 to a suitable treating agent. Nor is it limited to any particular method of producing the desired pressure of dissociation of the agent employed. In many cases a gaseous agent already having the desired oxygen 85 pressure may be available, as, for example, the gases emanating from the stack of an iron producing furnace, or such gases may be modified in a manner to give the desired oxygen pressure. 90

The critical temperatures of some of the metals with respect to other oxidizable elements with which they are commonly associated are known. However, in case such temperature for any required metal or metals is not known, a suitable working temperature can readily be ascertained by blowing samples of the material to be treated at successively progressing temperatures with air 95 or oxygen. By comparing the relative oxidation of the different elements of such treated samples a temperature can be determined at which the element or elements to be eliminated from the metal have a stronger affinity for oxygen than has the metal which it is desired to retain unoxidized. Having thus or in any other manner ascertained a 100 suitable working temperature, a gaseous mixture having oxidizing properties with respect to the substances to be eliminated 105 from the metal and having non-oxidizing properties with respect to the metal itself 110 can readily be determined. A suitable gaseous mixture can best be selected by mixing with a reducing gas, as for example carbon 115 monoxid (CO), a gas having oxidizing properties, as for example carbon dioxid (CO<sub>2</sub>), and treating samples of the material to be refined, maintained at the working 120 temperature previously ascertained in the 125

temperature previously ascertained in the 130

above described manner, with such progressively enriched gaseous mixtures. Such treatment should be thorough and should be prolonged beyond the point at which the 5 undesired elements are eliminated from the metal. From among those of the gaseous mixtures which do not oxidize, even with prolonged treatment at the selected temperature, the metal which it is to retain unoxidized, a mixture should be selected which 10 oxidizes the undesired components of the material, and preferably that mixture having the strongest oxidizing action at the selected temperature on said undesired components. In such manner a suitable working 15 temperature and a gaseous mixture suitable for treating the material at such temperature can readily be ascertained.

My invention as applied to the removal of 20 phosphorus may be further illustrated by a concrete example of the character of the material under treatment, the temperature at which it is maintained, and a gaseous mixture that will provide a suitable oxygen 25 pressure at such temperature. With a charge consisting of Bessemer steel and a lime flux, maintained at a temperature of approximately 1700° C., a gaseous mixture containing 23% of carbon monoxid (CO), 30 12% of carbon dioxid (CO<sub>2</sub>), and 1% of oxygen (O) will at approximately atmospheric pressure, satisfactorily eliminate phosphorus and sulfur without danger of overblowing the iron. Such a gas at a temperature 35 of 1700° C., will have an oxygen pressure of approximately 38 mm. of mercury. By actual test, under the above conditions, I have reduced phosphorus in Bessemer steel from .096%, to .019%, and sulfur from .041% to .013%, without oxidizing 40 the iron. It will be understood that the above is but an example of one of the many gaseous mixtures that will according to my process accomplish the desired result. For 45 example, though I have found that carbon dioxid alone will oxidize iron at a temperature of 1300° C., a mixture containing 12% of carbon dioxid and 3% of carbon monoxid will keep the iron reduced. I have further- 50 more used a mixture containing from 6 to 8% of carbon monoxid and from 12 to 15% of carbon dioxid and found that with the bath maintained at a temperature of about 1350° C., the reducing agent carbon monoxid 55 was present in sufficient quantity to prevent the oxidization of iron or manganese and yet that the mixture was oxidizing with respect to phosphorus. In the examples given the percentages are stated in volumes and the remaining portion of the mixture 60 may consist of some inert gas, such as nitrogen.

It is apparent that the process broadly is applicable not only to the removal of phosphorus and sulfur, but also to the removal of

other elements. Such broad features of my invention and certain other specific embodiments thereof are described in my co-pending applications, Serial No. 470,921 filed Jan. 6, 1909, Serial No. 488,360 filed Apr. 7, 70 1909, and Serial No. 531,529 filed Dec. 6, 1909.

I claim:—

1. The process of refining metals and alloys containing phosphorus as an impurity, 75 which consists in heating the material under treatment to a temperature at which the oxygen - affinity of phosphorus is greater than that of the element or elements to be retained, and in subjecting the heated material to the action of a gaseous mixture containing an oxygen-compound having a pressure of dissociation suitable, at a temperature of the heated material, for oxidizing phosphorus but unsuitable for like action 80 upon the element or elements which it is desired to retain unoxidized. 85

2. The process of refining metals and alloys containing phosphorus as an impurity, 90 which consists in heating the material under treatment, in the presence of a flux suitable for forming a slag with oxidized phosphorus, to a temperature at which the oxygen-affinity of phosphorus is greater than that of the element or elements to be retained, and in subjecting the heated material to the action of a gaseous mixture containing an oxygen - compound suitable, at the temperature of the heated material, for oxidizing phosphorus but unsuitable or like 95 action upon the element or elements which it is desired to retain unoxidized. 100

3. The process of refining metals and alloys containing phosphorus and sulfur as impurities which consists in heating the material under treatment, in the presence of a flux suitable for forming a slag with phosphorus and sulfur, to a temperature at which the oxygen-affinity of phosphorus is greater than that of the element or elements 105 to be retained, and in subjecting the heated material to the action of a gas containing carbon dioxid mixed with carbon monoxid in proportions suitable for oxidizing phosphorus but unsuitable for a like action upon 110 the element or elements which it is desired to retain unoxidized. 115

4. The process of purifying phosphorus-bearing iron, which consists in maintaining, in a furnace, a molten bath of the material 120 under treatment at a temperature at which the oxygen pressure of oxid of iron is higher than the oxygen pressure of oxid of phosphorus, and in subjecting the molten bath to a gaseous oxidizing agent having an oxygen pressure intermediate said aforesigned oxygen pressures. 125

5. The process of producing steel from an iron alloy containing phosphorus, which consists in maintaining in a furnace a 130

molten bath of the alloy at a temperature at which the oxygen pressure of oxid of iron is higher than the oxygen pressure of oxid of phosphorus, and in subjecting the molten bath to a gaseous oxidizing agent having an oxygen pressure suitable for the selective oxidation of the phosphorus of the bath.

6. The process of producing steel from an iron alloy containing phosphorus, which 10 consists in maintaining, in a furnace, a molten bath of the alloy at a temperature at which the oxygen pressure of oxid of iron is higher than the oxygen pressure of oxid of phosphorus and in subjecting the molten bath, in the presence of a flux suitable for forming a slag with oxidized phosphorus, to a gaseous oxidizing agent having an oxygen pressure intermediate said aforesaid oxygen pressures.

20 7. The process of refining an iron alloy containing phosphorus and sulfur as impurities, which consists in maintaining in a furnace a molten bath of the mixture at a temperature at which the oxygen pressure of oxid of iron is higher than the oxygen pressure of oxid of phosphorus, and in subjecting the molten bath to a gaseous oxidizing agent having an oxygen pressure suitable for the selective oxidation of the phosphorus 30 of the bath.

8. The process of refining an iron alloy containing phosphorus and sulfur as impurities, which consists in maintaining in a furnace a molten bath of the mixture at a 35 temperature at which the oxygen pressure of oxid of iron is higher than the oxygen pressure of oxid of phosphorus, and in subjecting the molten bath to a gaseous oxidizing agent having an oxygen pressure intermediate 40 ate said aforesaid oxygen pressures.

9. The process of refining an iron alloy containing phosphorus and sulfur as impurities, which consists in maintaining in a furnace a molten bath of the mixture at a 45 temperature at which the oxygen pressure of oxid of iron is higher than the oxygen pressure of oxid of phosphorus, melting with the bath a flux high in lime, and in subjecting the molten bath to a gaseous oxidizing agent 50 having an oxygen pressure suitable for the selective oxidation of the phosphorus of the bath.

10. The process of refining an iron alloy containing phosphorus and sulfur as impurities, which consists in maintaining in a 55 furnace a molten bath of the mixture at a temperature at which the oxygen pressure of oxid of iron is higher than the oxygen pressure of oxid of phosphorus at that temperature, melting with the bath a flux suitable

for forming a slag with oxidized phosphorus and also suitable for taking up sulfur from the bath, and in subjecting the molten bath to a gaseous oxidizing agent having an oxygen pressure suitable for the selective oxidation 65 of the phosphorus of the bath.

11. The process of refining metals and alloys containing an impurity which when oxidized is capable of forming a slag with a fluxing agent, said process consisting in 70 maintaining the material under treatment at a temperature at which the oxygen pressure of the oxid of the element which is to be retained is higher than the oxygen pressure of the oxid of the impurity, and in subjecting the material, in the presence of the flux suitable for forming a slag with the oxidized impurity, to a gaseous oxidizing agent having an oxygen pressure intermediate 75 the said aforesaid oxygen pressures. 80

12. The process of refining metals and alloys, containing an impurity which when oxidized is capable of forming a slag with a fluxing agent, said process consisting in maintaining, in a furnace, a molten bath of 85 the metal or alloy at a temperature at which the oxygen pressure of the oxid of the metal is higher than the oxygen pressure of the oxid of the impurity, and in subjecting the molten bath, in the presence of a flux suitable for forming a slag with the oxidized impurity, to a gaseous agent having oxidizing properties with respect to said impurity and reducing properties with respect to 90 oxides of the metal. 95

13. The process of refining metals and alloys, containing an impurity which when oxidized is capable of forming a slag with a fluxing agent, said process consisting in heating the material under treatment, in 100 the presence of a flux suitable for forming a slag with the oxidized impurity, to a temperature at which the oxygen-affinity of said impurity is greater than the oxygen-affinity 105 of the element or elements to be retained, and in subjecting the heated material to the action of a gas containing carbon dioxide mixed with carbon monoxide in proportions such that the gaseous mixture has, at the 110 temperatures of treatment, oxidizing properties with respect to said impurity and reducing properties with respect to oxides of such element or elements to be retained.

In witness whereof, I hereunto subscribe my name this twentieth day of July A. D., 115 1908.

ALBERT E. GREENE.

Witnesses:

CLARA P. CLARK,  
CATHERINE MORGAN.